

1

3,752,697

## TREATMENT OF CELLULOSIC FIBER CONTAINING FABRICS TO IMPROVE THE PHYSICAL CHARACTERISTICS

Angelo J. Ramunda, deceased, late of Fairlawn, N.J., by  
Phyllis G. Ramunda, executrix, Fairlawn, N.J., Phillip  
Adams, Murray Hill, Sidney Beinfest, Berkeley Heights,  
and Thaddeus A. Gulakowski, Ridgefield, N.J., assignors to Millmaster Onyx Corporation, New York, N.Y.  
No Drawing. Continuation-in-part of abandoned application Ser. No. 789,916, Jan. 8, 1969. This application May 19, 1971, Ser. No. 145,042

Int. Cl. D06m 13/12

U.S. Cl. 117—138.8 F

5 Claims

### ABSTRACT OF THE DISCLOSURE

A treatment for cellulosic fabrics and fabrics constructed of blends of cellulosic and non-cellulosic synthetic fibers, whereby the durability of the fabrics is retained even after repeated launderings while the "hand" of the fabrics is much improved over that obtained by prior treatments. This treatment consists of the application to the fabrics of a composition containing, as the active ingredient, a mixture of methylolated methyl carbamate with either (a) methylolated methoxyethyl carbamate, or (b) methylolated hydroxyethyl carbamate, or (c) methylolated n-propyl carbamate wherein the percentage of the methylolated methyl carbamate is about from 10 to 70 mol percent and of the other component is between about 90 to 30 mol percent.

This is a continuation-in-part of copending application Ser. No. 789,916, filed Jan. 8, 1969, now abandoned. This invention relates to a method and composition for treating textiles, and it particularly relates to the treatment of fabrics made from cellulosic fibers or blends of cellulosic and non-cellulosic synthetic fibers for the purpose of providing satisfactory "durability" (ability to withstand abrasion, stretch, strain, etc.) as well as providing a very good "hand," after repeated launderings.

It has heretofore been proposed to utilize a mixture of methylolated n-propyl and isopropyl carbamate resins for the present purpose. However, although the "wash-wear" and "durability" properties of such compositions were, in general, highly satisfactory, it was found that the "hand" of the treated fabrics was somewhat "papery" was unpleasant to the touch. This "hand" was greatly improved by the compositions of the present invention. Furthermore, the isopropyl carbamate component is quite costly.

It is known that methylolated methyl carbamate will generally provide satisfactory results in the treatment of textile fabrics. However, it has been found that the use of such methylolated methyl carbamates, by themselves, is objectionable because it results in a fishy odor or in other odors such as that of formaldehyde. This odor can only be eliminated by after-washing the cured fabric. Furthermore, methylolated methyl carbamates, by themselves, cause the development of discoloration when subjected to the customary high temperatures used in short-time curing operations.

In accordance with the present invention, it has now surprisingly been discovered that mixtures of methylolated methyl carbamate with either methylolated methoxyethyl carbamate, methylolated hydroxyethyl carbamate, or methylolated propyl carbamate, and preferably the latter, wherein the percentage of the methylolated methyl carbamate is in the range of about 10-70%, preferably 40-60% of the mixture, and the percentage of the other component is in the range of about 30 to 90 mol percent, results in a composition which may be applied to fabrics and cured at either the normal high temperatures or at

2

lower temperature over longer periods, without discoloration or the development of objectionable odors. At the same time, very satisfactory "wash-wear," "durability" and "hand" properties are retained. These advantages are, furthermore, obtained without extra processing steps.

It is possible to prepare the several methylolated carbamates separately, and combine them in the required proportions; or the methyl carbamate may be mixed with either n-propyl carbamate, hydroxyethyl carbamate, or methoxyethyl carbamate, and the mixture then methylolated together, as described in the following examples. There are advantages, for example, in employing certain mixed carbamates which are liquid, although their components are solid, as disclosed in U.S. Pat. No. 3,014,807. These mixtures may be used as such, or they may be used along with a sufficient quantity of ether component to arrive at the desired mol ratio.

The following examples are illustrative of the invention, with no intent, however, to limit the invention except as claimed:

### EXAMPLE 1

An agitated three-necked flask, fitted with a thermometer and a reflux condenser, was charged with 75 grams (one mol) of methyl carbamate, 103 grams (one mol) of n-propyl carbamate, 324 grams (four mols) of 37% aqueous formaldehyde, 243 grams of water, and a requisite amount of 25% aqueous NaOH to bring the pH to  $10.0 \pm .05$ . The mixture was maintained at  $50-53^\circ\text{C}$ , under agitation, at atmospheric pressure, for four hours, or until the reaction was complete. The product consisted largely of the dimethylol derivatives of the alkyl carbamate mixture. The pH was then reduced to 6.0-6.5 by the careful and gradual addition of concentrated hydrochloric acid.

The mol ratio of dimethylolmethyl carbamate to dimethylol-n-propyl carbamate was therefore 1:1, and the active content was 40% by weight as dimethylol alkyl carbamates.

### EXAMPLE 2

In the same manner as in Example 1, 90 grams (1.2 mols) of methyl carbamate, 82.4 grams (0.8 mol) of n-propyl carbamate, 324 grams (four mols) of 37% aqueous formaldehyde and 235 grams of water were reacted. The mol ratio of methylolated methyl to n-propyl carbamates was therefore, 1.5:1, and the active content was 40% by weight.

### EXAMPLE 3

Similarly to Example 1, 60 grams (0.8 mol) of methyl carbamate and 123.6 grams (1.2 mols) of n-propyl carbamate were reacted with four mols of aqueous formaldehyde in 251 grams of water. The ratio of methylolated methyl carbamate to n-propyl carbamate was therefore 1:1.5. The active content of dimethylolated carbamates was 40% by weight.

### EXAMPLE 4

In the manner of Example 1, a 40% active solution of a dimethylolated 50:50 mixture of methyl carbamate and methoxyethyl carbamate was prepared. Instead of an equimolar mixture, any desirable proportion may be dimethylolated in the same way. The same solution may be prepared using hydroxyethyl carbamate instead of the methoxyethyl carbamate.

The products of Examples 1, 2, 3 and 4 and also, as controls, 40% aqueous solutions of the corresponding dimethylol derivatives of n-propyl carbamate and of methoxyethyl carbamate (about 52:48) were applied to fabrics of cotton broadcloth, cotton twill and 65/35 Dacron polyester/cotton broadcloth by padding them in a bath containing 22.5 parts by weight of the respective methylolated carbamate (hereinafter referred to as "re-

actant") and a mixed zinc-magnesium salt catalyst, in the parts by weight indicated in each case in the following tables, the balance being water.

Although the mixed zinc-magnesium salt catalyst used

- (2) Wash/wear rating (1 wash and 5 washes)—  
AATCC Method No. 88-B-1964T  
(3) Chlorine, retained, damage by, single sample method, percent—AATCC Method No. 92-1962.

TABLE I

[Fabric: 100% cotton broadcloth. Catalyst: 4%. Wet pickup: 55-65%. Cure: "A"—270-300° F., two minutes. "B"—340° F., two minutes.]

| Reactant    | Cure | Tensile | Tear | Flex abrasion | CAR° | W./W.  |          | Cl. ret. percent loss |
|-------------|------|---------|------|---------------|------|--------|----------|-----------------------|
|             |      |         |      |               |      | 1 wash | 5 washes |                       |
| Pr.....     | A    | 33      | 512  | 223           | 229  | 3.3    | 3.2      |                       |
| Pr.....     | B    | 27      | 320  | 136           | 257  | 3.9    | 3.7      | 4.2                   |
| MBC.....    | A    | 33      | 498  | 231           | 227  | 3.3    | 3.1      |                       |
| MBC.....    | B    | 27      | 336  | 138           | 262  | 4.2    | 4.1      | 2.1                   |
| 1:1.....    | A    | 34      | 464  | 242           | 239  | 3.5    | 3.2      |                       |
| 1:1.....    | B    | 28      | 320  | 130           | 260  | 3.9    | 3.8      | 2.0                   |
| 1.5:1.....  | A    | 31      | 480  | 225           | 235  | 3.4    | 3.3      |                       |
| 1.5:1.....  | B    | 26      | 288  | 143           | 258  | 4.0    | 4.0      | 3.3                   |
| 1:1.5.....  | A    | 32      | 480  | 237           | 235  | 3.5    | 3.3      |                       |
| 1:1.5.....  | B    | 26      | 320  | 127           | 261  | 4.0    | 3.7      | 6.3                   |
| Me/MEC..... | A    | 33      | 490  | 221           | 249  | 3.5    | 3.5      |                       |
| Me/MEC..... | B    | 27      | 310  | 139           | 261  | 3.2    | 3.1      | 1.5                   |

NOTE.—Shrinkages were acceptable for all samples. Chlorine damage was evaluated after five commercial launderings with acid sour, using zinc silicofluoride. No discoloration was noted on any sample after chlorination and subsequent scouring.

in this example is preferred, other catalysts may be substituted. As, for example, the chloride, nitrate, sulfates and fluoborate salts of Group II elements, such as magnesium and zinc.

#### EXAMPLE 5

In the manner of Example 1, dimethylolated methyl-, n-propyl- and -methoxyethyl carbamates were prepared singly and separately, and finished at 40% activity by weight. Mixtures of the methylolated methyl carbamate were then prepared with each of the above homologs in the desired mol ratios.

It is to be understood that "40% activity by weight" is merely a matter of convenience, and other concentrations may be prepared within reasonable limits in order to facilitate the preparation of textile treating baths, with or without the addition of auxiliaries.

In the following tables, the n-propyl carbamate reactant is abbreviated to "Pr"; the methoxyethyl carbamate reactant is abbreviated to "MEC"; the products of Examples 1, 2 and 3 are designated by their respective ratios of methyl to propyl components, i.e., 1:1, 1.5:1 and 1:1.5; the mixture of methyl and methoxyethyl is indicated as "Me/MEC."

For the purpose of comparing these reactants, other auxiliaries frequently used, such as lubricants, softeners, wetting agents and resinous materials which contribute to such desirable qualities as "hand," "durability" and the like, have been omitted. The properties listed in the following tables are therefore dependent only on the basic components of this invention and not on the inclusion of any additives. It will, therefore, be appreciated that these listed properties may be, in some cases at least, significantly enhanced by the inclusion of such auxiliaries.

In each case, the fabric was padded in the bath to the indicated wet pickup, dried for a period of between about two and four minutes at a temperature of between about 250° F. and 350° F., and cured for a period of between one-half minute and two minutes at a temperature of between about 300° F. and 400° F.

The following testing methods were used in the examples given hereinafter:

From the Federal Specification, Textile Test Methods:

- (1) Tensile strength (pounds, fill)—Method CCC-T-191B-5102
- (2) Tearing strength (grams, fill)—Method CCC-T-191B-5132
- (3) Flexing abrasion resistance (1/2" x 2", fill)—Method CCC-T-191B-5300

From the 1964 Technical Manual of the American Association of Textile Chemists and Colorists:

- (1) Crease-angle retention rating (warp+fill)—AATCC Method No. 88-C-1964T

The range of 40%–60% for Me/Pr in the above table, the preferred range, shows no significant variation. The same is true for Me/MEC, which is reported above for 50/50 composition only.

TABLE II

[Fabric: 100% cotton twill. Catalyst: 5.5%. Wet pickup: 55-70%. Cure: "A"—270-300° F., two minutes. "B"—340° F., two minutes.]

| Reactant    | Cure | Tensile | Tear | Flex abrasion | CAR° | W./W.  |          | Cl. ret. percent loss |
|-------------|------|---------|------|---------------|------|--------|----------|-----------------------|
|             |      |         |      |               |      | 1 wash | 5 washes |                       |
| Pr.....     | A    | 51      | 832  | 274           | 248  | 4.3    | 3.9      |                       |
| Pr.....     | B    | 43      | 704  | 253           | 261  | 3.9    | 3.9      |                       |
| MEC.....    | A    | 53      | 960  | 281           | 260  | 4.3    | 3.2      |                       |
| MEC.....    | B    | 43      | 960  | 247           | 262  | 4.3    | 4.9      |                       |
| 1:1.....    | A    | 51      | 960  | 208           | 242  | 4.2    | 4.9      |                       |
| 1:1.....    | B    | 38      | 928  | 259           | 254  | 4.2    | 4.9      |                       |
| 1.5:1.....  | A    | 48      | 896  | 265           | 259  | 4.2    | 3.2      |                       |
| 1.5:1.....  | B    | 46      | 768  | 233           | 265  | 4.0    | 4.0      |                       |
| 1:1.5.....  | A    | 54      | 832  | 293           | 246  | 4.0    | 4.0      |                       |
| 1:1.5.....  | B    | 43      | 896  | 277           | 267  | 4.0    | 4.0      |                       |
| Me/MEC..... | A    | 49      | 940  | 296           | 252  | 4.2    | 4.0      |                       |
| Me/MEC..... | B    | 43      | 926  | 250           | 250  | 4.1    | 4.0      |                       |

NOTE.—Shrinkage in every case was less than 1%. The range of 40%–60% for Me/Pr in the above table, the preferred range, shows no significant variation. The same is true for Me/MEC, which is reported above for 50/50 composition only.

TABLE III

[Fabric: 65/35 Dacron/cotton broadcloth. Catalyst: 7%. Wet pickup: 55-60%. Cure: "A"—340° F., three minutes. "B"—400° F., thirty seconds.]

| Reactant    | Cure | Shrinkage, warp+fill |          | CAR° | W./W.  |          | Cl. ret. percent loss |
|-------------|------|----------------------|----------|------|--------|----------|-----------------------|
|             |      | 1 wash               | 5 washes |      | 1 wash | 5 washes |                       |
| Pr.....     | A    | 0.5-0                | 0.5-0    | 283  | 4.1    | 4.1      |                       |
| Pr.....     | B    | 1.0-0                | 1.0-0    | 293  | 4.3    | 4.2      |                       |
| MEC.....    | A    | 1.0-0                | 1.0-0    | 282  | 4.3    | 4.0      |                       |
| MEC.....    | B    | 0.5-0                | 1.0-0    | 291  | 4.4    | 4.2      |                       |
| 1:1.....    | A    | 0.5-0                | 1.0-0    | 281  | 4.2    | 4.2      |                       |
| 1:1.....    | B    | 0.5-0                | 0.5-0    | 291  | 4.4    | 4.3      |                       |
| 1.5:1.....  | A    | 1.0-0                | 1.0-0    | 280  | 4.2    | 4.2      |                       |
| 1.5:1.....  | B    | 0.5-0                | 0.5-0    | 294  | 4.4    | 4.3      |                       |
| 1:1.5.....  | A    | 0.5-0.5              | 0.5-0.5  | 280  | 4.1    | 4.0      |                       |
| 1:1.5.....  | B    | 1.0-0                | 1.0-0.5  | 294  | 4.4    | 4.3      |                       |
| Me/MEC..... | A    | 0.5-0                | 0.5-0    | 280  | 4.2    | 4.0      |                       |
| Me/MEC..... | B    | 1.0-0                | 0.5-0    | 287  | 4.3    | 4.2      |                       |

NOTE.—Color and odor were good for all samples. The range of 40%–60% for Me/Pr in the above table, the preferred range, shows no significant variation. The same is true for Me/MEC, which is reported above for 50/50 composition only.

65 The above examples and data tables include mixtures of methyl and methoxyethyl. Comparable results are also obtained when substituting hydroxyethyl for the methoxyethyl component.

70 Although the invention is described above with the utilization of methylolated methyl carbamate as one of the essential components, this being the preferred form of the invention, it is also possible, although least preferable at this time, to substitute methylolated hydroxyloweralkyl carbamates for the methylolated methyl carbamate; as for example, methylolated hydroxyethyl, methylolated hy-

droxy-n-propyl, methylolated hydroxyisopropyl or methylolated hydroxybutyl carbamate. In such case, of course, the methylolated hydroxyethyl carbamate cannot be used as the second component when it is used as the first component.

The invention claimed is:

1. A method of treating fabric which comprises applying to the fabric an aqueous composition consisting essentially of methylolated methyl carbamate in admixture with either (a) methylolated hydroxyethyl carbamate, 10 (b) methylolated methoxyethyl carbamate, or (c) methylolated n-propyl carbamate, wherein the percentage of the methylolated methyl carbamate is between about 10 to 70 mol percent and the percentage of the other component is between about 90 to 30 mol percent, drying 15 the treated fabric, and then curing the dried fabric.
2. The method of claim 1 wherein the percentage of the methylolated methyl carbamate is between about 40 to 60 mol percent.
3. The method of claim 1 wherein the drying is effected at a temperature of about 250° F. to 350° F., and the curing is effected at a temperature of about 300° F. to 400° F.
4. The method of claim 1 wherein the aqueous composition also includes an effective amount of a catalyst.

5

5. A fabric of cellulosic fibers or blends of cellulosic and non-cellulosic synthetic fibers, wherein the fabric is treated by the method of claim 1.

#### References Cited

##### UNITED STATES PATENTS

|           |         |                       |             |
|-----------|---------|-----------------------|-------------|
| 3,420,696 | 1/1969  | Cotton et al. _____   | 117—139.4 X |
| 3,416,880 | 12/1968 | Kullman et al. _____  | 8—116.3     |
| 3,219,632 | 11/1965 | Frick et al. _____    | 8—116.3 X   |
| 3,014,807 | 12/1961 | Beinfest et al. _____ | 106—162     |
| 3,565,680 | 2/1971  | Ramunda et al. _____  | 117—139.4 X |
| 3,454,423 | 7/1969  | Cohen et al. _____    | 117—139.5   |
| 3,402,989 | 9/1968  | Canter et al. _____   | 8—116.3     |
| 3,622,261 | 11/1971 | Cotton et al. _____   | 8—116.3 X   |
| 3,144,299 | 8/1964  | Frick et al. _____    | 8—116.3     |
| 3,424,724 | 1/1969  | Nordstrom _____       | 117—161 X   |
| 3,497,471 | 2/1970  | Cohen et al. _____    | 117—139.4 X |

20 WILLIAM D. MARTIN, Primary Examiner

H. J. GWINNELL, Assistant Examiner

U.S. CL. X.R.

25 117—139.4, 139.5 A, 143 A, 16 LN; 260—29.4 R